

July 28, 1936.

R. B. DAY

2,049,000

MANUFACTURE OF ASPHALT AND LUBRICATING OILS

Filed Feb. 26, 1934



Inventor:  
Roland B. Day,  
By: Spec. J. G. Gauj  
Attorney.

## UNITED STATES PATENT OFFICE

2,049,000

MANUFACTURE OF ASPHALT AND  
LUBRICATING OILS

Roland B. Day, Chicago, Ill., assignor to Universal  
Oil Products Company, Chicago, Ill., a cor-  
poration of Delaware

Application February 26, 1934, Serial No. 712,887

3 Claims. (Cl. 196—13)

This invention relates more particularly to the manufacture of asphalt and lubricating oils from cracked residua.

It is more specifically concerned with a process of treating cracked residua to increase the yield of asphalt and lubricating oils recoverable therefrom and combines a heat treatment under accurately controlled conditions along with the subsequent use of particular solvents for effecting segregation of the asphaltic and lubricating constituents.

The heavy tar-like residua produced in cracking and distilling operations vary in character to a considerable extent. They consist of mixtures of hydrocarbons of a definitely fluid character and compounds of a solid or semi-solid asphaltic character which may be looked upon as heavy hydrocarbon polymeric derivatives containing oxygen and sulphur which possess the commonly recognized characteristics of asphalts or pitches, that is, relatively high melting point, adhesiveness and a limited ductility. The physical properties of a cracked residuum such as viscosity, melting point, etc., and chemical properties such as tendency toward coking and resistance to oxidizing and weathering influences are determined by the character and relative amounts of their fluid and solid components.

A large number of cracked residua, particularly those which are the result of deep or intensive cracking to produce maximum yields of gasoline, approach a solid consistency at ordinary temperatures and have too high viscosity, too high fixed carbon content and too large a percentage of suspended cokey or carbonaceous material to permit their use as fuel oil in the ordinary type of atomizing burners. When employed directly as a road oil or asphalt, the presence of the fluid components of the mixture, which include some light oils and lubricating fractions of varying viscosity, renders their action under severe conditions uncertain, so that frequently heavy cracked residua are not suitable for such purposes.

The principal objects of the present invention are the production from cracked residua of maximum yields both of marketable asphalt and lubricating oil fractions, with the elimination of solid coke-like substances and light oils which have at the most only a fuel value.

In one specific embodiment the invention comprises the prolonged digestion of cracked residua at temperatures within the approximate range of 550 to 850° F., to effect substantial completion of polymerization reactions, followed by the

separate recovery from the polymerized material of asphalt and lubricating oil fractions by means of their differential solubility in selected solvents.

The sequence of steps by which the objects of invention are accomplished may be disclosed in connection with the description of a characteristic plant operation, and to assist in this description the attached drawing has been provided which shows diagrammatically in side elevation 10 and using conventional figures an arrangement of interconnected elements in which the process may be conducted.

Referring to the drawing line 1 containing control valve 2 indicates a supply line for cracked 15 residuum, which may come from intermediate storage or be supplied directly and continuously from a concurrently operating cracking plant. The first step of the process is necessarily a batch operation on account of the long period 20 of heating which has generally been found to be necessary for completing the polymerization reactions which were initiated in the cracking zone. While digester 3 is shown as a single unit 25 it represents any number of such units connected in parallel which may be employed in the first step of the process to insure a proper supply of polymerized residuum at all times for the succeeding steps of the process which are 30 preferably conducted continuously.

Digester 3 is positioned over a furnace 3' which is heated by the combustion of oil or other fluid fuel introduced to a burner by way of line 4 containing control valve 5. The digester is preferably insulated at all points except those immediately exposed to the hot combustion gases and the oil is maintained at the temperature of approximately 550 to 850° F., as previously stated. The exact temperature best for any given 35 residuum in consideration of the overall yields of asphalt and lubricating oil will be a matter of experiment, since the composition of cracked residua varies over a wide range depending upon the character of the original oil cracked, the 40 severity of temperature, pressure and time conditions imposed and special plant operating conditions. Moderate superatmospheric pressures up to approximately 100 pounds per square inch 45 may be employed with advantage in treating some residua.

During the digestion of the residuum a small amount of cracking may occur although the principal effect is the polymerization of the highly unsaturated constituents and the distillation of 5 relatively small amounts of low boiling distillates,

which leave the still through vapor line 6 containing control valve 7, and undergo refluxing in a tower 8. The fixed gases and low boiling vapors pass from the tower through a line 9 containing control valve 10, the vapors being condensed by condenser 11 and the liquid condensate and fixed gases following line 12 containing control valve 13 to enter a receiver 14 which is provided with a gas release line 15 containing a control valve 16 and a liquid draw line 17 containing a control valve 18. As already stated, the amount of distillate ordinarily produced during the digesting step (which is conducted at atmospheric or slightly superatmospheric pressure) is usually small and of the order of 5 to 10% by volume of the stock subjected to the digesting step. This distillate may be further fractionated to recover any gasoline boiling range fractions, the intermediate stocks being used as a light fuel or charging stock to the cracking plant.

After the period of digestion, which may range from 12 to 48 hours in different cases, the residuum is drawn from the digester, cooled to approximately atmospheric temperature and subjected to the action of selective solvents. As a rule the solvent extraction may be performed in one stage since the coke formed will settle quickly after the heat is taken from the bottom of the digester and a homogenous liquid is withdrawn for the solvent extraction. The solvent most generally preferred for the segregation of the asphaltic and lubricating constituents is a light paraffin naphtha of an average boiling point corresponding to a mixture of pentanes and hexanes, though if suitable equipment is provided to permit the use of pressure, butanes and propane may be used. The invention is not limited to the use of any particular class of solvents and may employ any single solvent or mixture of solvents which may be found suitable for effecting the desired results.

The fluid residuum is drawn from the digester through line 19 containing control valve 20 and transferred by a pump 21 by way of line 22 containing control valve 23 to a cooler 24 in which the temperature is only reduced to a point which will permit the use of the light solvent without undue losses and must not be brought too low in view of the tendency of the residuum to solidify or become too viscous for pumping. If desired, some of the solvent may be admitted at an intermediate point in the cooling coil.

The cooled residuum, with or without addition of a small amount of solvent, passes through line 25 containing control valve 26 and meets a stream of solvent from line 31 containing control valve 32. Line 31 is supplied with make-up solvent by way of line 28, control valve 29 and pump 30 and by recovered solvent from line 96, the production of which will be described in proper sequence. The volume of solvent used upon different pre-treated cracked residua will vary from approximately 0.5 to 2.0 volumes based on the volume of residuum though obviously this range of volumes is subject to great variations due to the differences in the character of the residua which may be treated and the different types of solvents which may be employed. When using an 86° A. P. I. paraffin naphtha the volume commonly employed is from 1.5 to 2.5 volumes per volume of residuum.

The residuum and solvent then pass through some type of mixing device indicated at 27 as a tube of moderate diameter containing filling or baffling material to create turbulence and then

pass through a line 26' containing a control valve 27' to a settling tank 33. In this tank zone 34 indicates an upper clear layer of a solution of oil in solvent, 35 indicates an intermediate zone containing suspended material and 36 a zone of settled asphalt. Settling drums of the type shown at 33 may be employed in parallel in case it is further necessary or expedient to warm the settled asphalt to insure sufficient fluidity for its ready pumping. If the material can be drawn continuously, parallel settlers may not be necessary. The settler is provided with a gas vent line 37 containing control valve 38 for the release of any fixed gas accumulations and this line may be connected to the solvent recovery vapor line 15 if desired although this is not shown in the drawing.

The settled asphalt, mixed with a certain amount of adhering solvent and oil may be drawn through a line 39 containing control valve 40 to a pump 41 and subjected to any further processing steps necessary for the production of a finished product. Ordinarily this will consist in simply distilling off any solvent or oil. Thus pump 41 discharging through line 42 containing control valve 43 may pass the asphalt through a tubular heating element 44 disposed to receive heat from a furnace 45, the heated material passing to line 46 containing control valve 47 to a fractionator 48. The conditions of distillation in this tower are so controlled that the solvent and light oils are driven off to pass through vapor line 49, control valve 50, condenser 51, line 52 and control valve 53 to a receiver 54 which is provided with the customary gas release line 55 containing control valve 56 and liquid draw line 57 containing control valve 58. If found expedient the liquid products may be worked up for solvent recovery and added to the main body of solvent distilled from the liquid oil solution.

The asphalt constituting one of the major products of the process passes through line 59 containing control valve 60 to a receiver 61 which is again provided with a customary gas release line 62 containing control valve 63 and a liquid draw line 64 containing control valve 65 leading to some intermediate storage. Depending upon the temperature employed in the fractionator, this may be a product of varying consistency. It may be subjected to any further refining steps necessary for producing a finished material.

For the recovery of lubricating oil stocks the upper clear layer 34 in settler 33 is removed by way of line 66 containing control valve 67, taken by pump 68 and discharged by way of line 69 containing control valve 70 through the solvent recovery plant comprising heating element 71 and a subsequent fractionator 75. The heating unit 71 is disposed to receive heat from furnace 72 and the products are discharged by way of line 73 containing control valve 74 at a temperature sufficient to enable the recovery of the solvent as an overhead vapor and the lubricating stocks as a tower reflux, the latter passing out through draw line 86 containing control valve 87 to receiver 88 provided with a gas release line 89 containing control valve 90 and a liquid draw line 91 containing control valve 92. Stocks produced at this point may be worked up into finished lubricating oils in any desired manner such as, for example, vacuum distillation to produce cuts of different viscosities, solvent extraction, sulphuric acid treatment, chilling and pressing to remove paraffin or treatment with clay to improve color.

Solvent vapors from fractionator 15 pass 71

through vapor line 76 containing control valve 77 and are condensed during passage through condenser 78 from which they flow through line 79 containing control valve 80 to receiver 81 provided with a fixed gas release line 82 containing control valve 83 and a liquid draw line 84 containing control valve 85.

In the usual operation of the process all the overhead produced at this point will be returned to the solvent extraction step by way of a line 93 containing control valve 94, a recirculating pump 95 and a discharge line 96 containing control valve 97 and leading to solvent line 31 previously described.

The following example is given to show the general character of the results obtainable by the use of the process, and while it is entirely representative, it is only one of a large number and the scope of the invention is not limited by the specific data given.

A Mid-Continent cracked residuum having an A. P. I. gravity of 8.9° was digested for 24 hours at a temperature of 700° F., and a pressure of 50 pounds per square inch. Following the digestion the residuum was cooled and mixed with approximately 2 volumes of a close-cut paraffinic distillate fraction having the approximate boiling range of pentane. The soluble and insoluble materials were separated and worked up according to the general process outlined in connection with the drawing and the following table shows the comparison between the yields of various products obtained from the untreated and the treated residuum by the solvent extraction step.

|                                                              | Untreated residuum | Treated residuum |
|--------------------------------------------------------------|--------------------|------------------|
| Percent asphalt by pentane precipitation                     | 12                 | 42               |
| Percent wax by chilling to -20° F. in 1-1 volumes in pentane | 10                 | 8                |
| Percent overhead at 500° F.                                  | 5                  | 15               |
| Percent of 100 V. I. finished lubricating oil                | 16                 | 23               |
| Percent heavy unsaturated oils                               | 57                 | 9                |

An inspection of the data reveals the fact that the asphalt content has been increased, the paraffin content slightly decreased, and the lubricating oil fraction increased by a considerable percentage. The increase of overhead at 500° F. from 5 to 15% indicates a slight cracking and it is evident from the decided drop in the percentage of heavy unsaturated oils from 57% to 9% that they have been converted into the asphalt and lubricating oil fractions. The asphalt produced by the polymerizing step compared either with the asphalt recoverable by solvent action from the untreated residuum or with asphalt of corresponding penetration prepared from straight run residuum has a much lower susceptibility factor, that is, there is less change

in penetration, melting point and ductility as temperatures are increased.

The character and value of the invention is obvious from a consideration of the preceding specification and single instance of results obtained, but neither is to be construed as imposing undue limitations upon its scope.

I claim as my invention:

1. A process for the treatment of liquid residue from a hydrocarbon cracking process which comprises, subjecting said residue to prolonged digestion at temperatures within the approximate range of 550° F. and 850° F., under non-hydrogenating conditions and without substantial cracking thereof, to effect polymerization reactions and to increase the asphalt and lubricating oil content thereof, subjecting the thus treated cracked residue to the action of a solvent, separating the undissolved material comprising asphalt from the supernatant liquid from which asphaltic components have been separated, and removing and recovering the solvent and the dissolved oil by distillation of the solvent.

2. A process for the treatment of liquid residue from a hydrocarbon cracking process which comprises, subjecting said residue to prolonged digestion at temperatures within the approximate range of 550° F. and 850° F., under non-hydrogenating conditions and without substantial cracking thereof, to effect polymerization reactions and to increase the asphalt and lubricating oil content thereof, subjecting the thus treated cracked residue to the action of a solvent, comprising a relatively low-boiling hydrocarbon separating the undissolved material comprising asphalt from the supernatant liquid from which asphaltic components have been separated, and removing and recovering the solvent and the dissolved oil by distillation of the solvent.

3. A process for the treatment of liquid residue from a hydrocarbon cracking process which comprises, subjecting said residue to prolonged digestion at temperatures within the approximate range of 550° F. and 850° F., under non-hydrogenating conditions and without substantial cracking thereof, to effect polymerization reactions and to increase the asphalt and lubricating oil content thereof, subjecting the thus treated cracked residue to the action of a solvent, comprising a relatively low-boiling hydrocarbon, separating the undissolved material comprising asphalt from the supernatant liquid from which asphaltic components have been separated, removing and recovering the solvent and the dissolved oil by distillation of the solvent, and producing lubricating oil from the dissolved oil by subjecting the same to chemical treatment.

ROLAND B. DAY.